

May 31, 1932.

H. J. BRUNK

1,861,298

BLUE PRINT AND PROCESS OF MAKING THE SAME

Filed May 11, 1931



Inventor

Harold J. Brunk,

George Bayard Jones, Atty.

Witness:

Chas. L. Townsend

## UNITED STATES PATENT OFFICE

HAROLD J. BRUNK, OF CHICAGO, ILLINOIS, ASSIGNOR TO THE C. F. PEASE COMPANY, A CORPORATION OF DELAWARE

## BLUE PRINT AND PROCESS OF MAKING THE SAME

Application filed May 11, 1931. Serial No. 536,378.

This invention relates to improvements in blueprints and in the process of making the same, i. e., paper which has a sensitized coating applied thereto and after exposure 5 to light, with a tracing or negative against the coated side and toward the light source, is developed, resulting in a blue sheet with white lines on it, or a white sheet with blue lines on it.

10 The coating is applied as a solution containing mixtures of potassium ferricyanide and organic salts of iron such as ferric ammonium oxalate. During the period of exposure to such light the potassium ferricyanide is partly reduced to potassium ferrocyanide while the ferric ammonium oxalate is reduced to ferrous ammonium oxalate.

After exposure, the paper is washed with clear water which removes all the unexposed chemical from the areas which were 20 behind the opaque portion of the tracing or negative and also removes the loose exposed or reduced chemical, i. e., that portion which does not adhere to the fibres of the paper.

25 This washing, in a certain sense, also starts the process of oxidation of the reduced chemical which action is necessary in the formation of the blue lines or areas. In other words, if left long enough in the water the so-called "potash" treatment hereinafter referred to, is unnecessary. It is the practice, however, to complete the oxidation by applying bichromate of potash or some other 30 strong oxidizing agent to the surface of the paper immediately after the application of the first water wash. The excess bichromate or "potash" must be washed off the surface by applying a second water wash, after which the paper is ready for drying.

40 Prints made in this manner are far from satisfactory or dependable when first class blueprints with clear white lines or blue line prints on a clear white background are desired. The difficulties may be analyzed as 45 follows:

When making blue line prints or blue lines on a white background from negatives of tracings, the fully exposed chemical in the area outside of or between negatives runs down into the white background and stains it blue immediately when water is applied 50 to the surface of the paper.

The blue lines themselves at certain exposures run down into the white ground giving them a ragged appearance.

55 In the case of blue prints, or white lines on a blue ground (which are obtained when a tracing or positive original is used) the blue in the ground runs over the line giving it a bluish cast and at the same time closing up on the line making it narrower than the line on the original tracing and at full exposures of the blue ground the line may be lost completely.

60 Due to the fact that this running of the blue takes place at or near the point of full exposure or reduction by light it is customary to make prints under-exposed with the idea of eliminating this "burning out" 65 of the white lines as it is commonly called. In making prints under-exposed or only partially reduced the deep Prussian blue color desired is never obtained; therefore, seldom, if ever, is the chemical on the paper changed 70 to the color it is capable of producing.

75 In trying to avoid this undesirable "running" at the sacrifice of color, the operator is forced to operate the printing machine within very close limits of speed or exposure time, which fact necessitates the preparation 80 of sensitized paper of several printing speeds when covering the range of average printing—which is from six inches to twelve feet per minute.

85 Various methods of washing have been tried with the idea of preventing this "running" or "bleeding" mentioned above but none has proven successful heretofore. No method of changing the application of water 90 is successful because the "bleeding" is caused

by the formation of insoluble Prussian blue when the unexposed chemical on the print mixes with or combines with the exposed or reduced portions. The Prussian blue 5 formed, runs into the white and cannot be washed out, once it stains the print. From this it is evident that moisture applied to the paper in a quantity sufficient to remove the surplus chemical, regardless of how applied, 10 is bound to cause the exposed chemical to mix with the unexposed portion, as nothing separates the two, and even if the blue formed is not in sufficient quantities to run very far, the line itself will be unsatisfactory.

15 The general object of the present invention is to overcome the foregoing difficulties by an improved process of developing the prints resulting in the elimination of "bleeding," regardless of the speed of operation of the 20 blueprint machine or of the length of exposure, and which also results in the production of clear white full lines on blueprints, a perfectly white background on blue line prints, a deep Prussian blue following full 25 exposures and one which does not fade readily, a wide range of exposure without the need of many different printing speeds and the successful printing from tracings or from negatives without changing the 30 speed.

A contributory object is to attain the foregoing advantages by developing the paper immediately after printing and before any 35 water has been applied to the surface, after which the prints are washed and may then be treated with an oxidizing agent.

Otherwise expressed, the present invention is directed to sensitizing paper with ferri 40 compounds, exposing the sensitized paper to a source of light with portions of the surface shielded from the source of light whereby the compounds of the exposed portion of the sensitized paper are reduced to a ferrous state. Thereafter, the paper is treated with 45 a developer containing ferric compounds adapted to render insoluble the reduced ferrous compounds and the so treated paper is then washed with water. Preferably the 50 ferri compounds of the developer are of the same chemical characteristics as the ferri compounds used to sensitize the paper.

More specifically, paper or other suitable material, is sensitized with a ferricyanide 55 and after exposure a reducing agent is used to convert the ferricyanide to ferrocyanide. The reducing agent at the same time is capable of forming with the reduced ferrocyanide a blue precipitate (Prussian blue) having 60 high tinctorial value. Any diffusion of the reduced ferrocyanide into the unexposed portions, such as would result in the formation of the same precipitate in the unexposed portions as is produced in the exposed portions, 65 is prevented by fixing, i. e., precipitating said

reduced ferrocyanide prior to washing with water.

A practical sensitizing formula is as follows: Potassium ferricyanide, 5 pounds in 5 gallons of water. Ferric ammonium oxalate, 34 pounds in 12½ gallons of water. Ammonium oxalate, 1¼ pounds in 4 gallons of water. Mix above together making a total batch of 21½ gallons of solution.

An appropriate developer for the above 75 would be: 1 pound potassium ferricyanide in 1 gallon of water. 5½ pounds ferric ammonium oxalate in 2 gallons of water. Mixing together gives 3 gallons of developer.

In the accompanying drawing I have illustrated a machine designed for carrying out the improved process.

Fig. 1 is a side elevation thereof;

Fig. 2 is an elevation of the opposite end of the developing attachment.

The frame of the machine 10 is similar to that of a well-known type of printing, washing and drying machine now on the market and since much of the mechanism is used in said commercial machine, except for the 80 means for applying the developing solution between the printing stage and the water washing stage, said machine will be described very briefly.

The sensitized paper is supported on a 85 suitable roller 11, at one end of the machine, the paper 12 being drawn past a sheet of curved glass 13, where it is exposed to a suitable source of light (preferably a row of arc lights) in a well-known manner, the paper 100 leaving the printing section of the machine where it passes over a roller 14 and then under a roller 15, the weight of which is supported in part by the loop of paper as shown, thereby maintaining the proper tension on the 105 paper and providing for expansion and contraction of the same.

The paper then passes the means for applying the developer which may have the form of a roll 16 dipping in a pan 17 containing a 110 developing solution supplied by a suitable reservoir 18.

This roll, pan and associated parts may be in the form of an attachment, readily applicable to existing machines.

From the developer the paper travels past the first water wash consisting of a tube 19 with suitable nozzles which direct sprays of water against the inclined surface of the paper in a manner which has been used heretofore, the paper thereafter travelling over suitable rollers to the "potash" roller 20 which dips in a pan 21, supplied with bichromate of potash or other suitable oxidizing agent, contained in a reservoir 22. The paper then travels upwardly past the final water wash, the water being supplied from the pipe 23, and thereafter passes through the dryer 24, where it is dried in the usual 130

manner, and thereafter wound on a removable roller 25.

The chemical mechanism of the process may be more fully appreciated by reference to the following diagrammatic scheme representing the composition of the chemicals on the paper in the unreduced (unexposed) and reduced (exposed) portions respectively;

10 Unreduced Reduced

Ferricyanide  $\left\{ \text{Fe}(\text{CN})_6 \right\}$  radical or ion  $\left\{ \text{Fe}(\text{CN})_6 \right\}$  radical or ion

Ferrocyanide

Ferric ( $\text{Fe}^{3+}$ ) radical cation

15 X represents the dividing line between the exposed and unexposed portions of the sensitized paper and it is an object of this invention to have this line sharply defined and prevent encroachment of the chemicals in the reduced area upon those of the unreduced area and vice versa.

In this diagram, only the more essential portions, i. e., ions or radicals of the reacting substances have been shown. For example, 25 potassium, sodium or other soluble ferricyanide may be used, the ferricyanide being the important consideration. This will be readily understood by those familiar with the 30 ionic theory or doctrine concerning which reference may be had to standard treatises on physical chemistry, e. g. "Physical Chemistry for Colleges" by Millard and "Theoretical Chemistry" by Noyes and Sherrill.

30 The photochemical reaction consists in the reduction of ferricyanide to ferrocyanide by the conjoint action of sunlight and a photo-sensitive reducing agent, as for example, an organic ferric salt broadly and, more specifically, ferric ammonium oxalate. There is no useful reaction between a ferric salt and a ferricyanide but a ferric salt and a ferrocyanide react to produce a deep blue 40 highly tinctorial water insoluble substance. In the old process the ferricyanide was reduced to ferrocyanide and the ferric salt to 45 ferrous salt in the exposed portions, and upon treatment with wash water a migration 50 over the line X took place, as shown by the arrows in the above diagram, resulting in an impairment or destruction of the highly desirable sharp definition between the exposed and unexposed portions.

55 The foregoing procedure prevents the combination on paper of (1) the ferrous ammonium oxalate and potassium ferricyanide that was not exposed to the light, in the course of printing, and (2) the potassium ferricyanide with any ferric ammonium oxalate that was not exposed to light in the course of printing. After developing as above, the prints are washed in a clear water wash and then completely oxidized with bichromate of potash or other agent, as previously

stated, and the surplus can then be washed off and the prints ready for drying.

The broad teaching of the present invention is that such migration or diffusion is prevented by fixing the reduced ferrocyanide before washing the paper. By this fixing process the ferrocyanide is rendered insoluble and incapable of reacting with the ferric salt in the unreduced portions. This fixing is carried out, as explained, by washing the paper with a solution of a ferric salt, containing ferric ( $Fe^{+++}$ ) ions, which reacts with the ferrocyanide in the exposed portions and converts it to insoluble ferric ferrocyanide. In those cases where a ferric organic salt is employed as the photosensitive reducing agent and is itself reduced to the ferrous condition, the fixing solution should also contain an agent, as for example a ferricyanide, to fix the ferrous salt and prevent it from diffusing and combining with ferricyanide in the unexposed portions.

Tests have been made with a large number of possible developers including all of the common ferric compounds and most of the rare and other metallic salts, from which the following show possibilities as developers: 90

### Potassium ferricyanide

### Ferric ammonium oxalate.

### Ferric-ammonium citrate.

### Ferric-sodium oxalate. Ferric oxalate.

### Ferric chloride.

### Ferric potassium oxalate.

### Sodium perborate.

The potassium ferricyanide and the ferric ammonium oxalate in combination are by far the best and the potassium ferricyanide works well alone on the slower printing papers. The relative amount of potassium ferricyanide and ferric ammonium oxalate can be changed to give different shades of blue, the deeper shades of blue being obtained when the relative amounts of potassium ferricyanide in the sensitizing formula and in the developing solution balance. For example, a fast printing paper has less potassium ferricyanide in the formula than a slow printing paper; therefore, less should be used in the developing solution.

In addition to potassium bichromate other oxidizing agents may be used, such as other bichromates, hydrogen dioxide, sodium perborate, potassium persulphate, and potassium ferricyanide. It is understood that the use of any of these agents follows the washing of the paper. Most of those listed as alternatives are too slow in their action for commercial use. For many purposes it is sufficient to wash the print and apply no further chemical treatment. In other words, the oxidation is not necessary, particularly if the machine is run slowly to give full reduction, in which case the bichromate of potash or equivalent may be omitted, although its use adds somewhat to the color.

The resulting prints constitute a remarkable improvement over blueprints and so-called white prints, and the like, made by the prevailing method, in that there is no running or "bleeding" of the blue line into the white areas at any speed or exposure, the blueprints show clear white full lines on a deep Prussian blue background, the blue line prints show a perfectly white background, the deep blue color fades slower than the present shades of blue when exposed to sunlight, and there is a wide range of exposure permissible which eliminates the need of providing sensitized papers with various different printing speeds.

It has been proposed heretofore to develop the unexposed portions of prints, i. e. the parts which were temporarily under the lines, which shielded them from the light. In the present invention, the exposed reduced portions of the prints are developed.

What I claim is:

1. The method of making non-bleeding photoprints comprising coating a sheet of material with a ferricyanide of an alkali metal and a light sensitive ferric ammonium compound of an organic acid, exposing portions of the coated surface to light, applying to said surface without preliminary watering a developer comprising a ferricyanide of an alkali metal and a ferric ammonium compound of an organic acid, and thereafter washing.

2. The method of making non-bleeding photoprints comprising coating a sheet of material with a ferricyanide of an alkali metal and a light sensitive ferric ammonium compound of a carboxylic acid, exposing portions of the coated surface to light, applying to said surface without preliminary watering a developer comprising a ferricyanide of an alkali metal and a ferric ammonium compound of a carboxylic acid, and thereafter washing.

45 3. The method of making non-bleeding photoprints comprising coating a sheet of material with potassium ferricyanide and ferric ammonium oxalate, exposing portions of the coated surface to light, applying to said surface without preliminary watering a developer comprising potassium ferricyanide and ferric ammonium oxalate, and thereafter washing.

4. The method of making non-bleeding photoprints comprising coating a sheet of material with potassium ferricyanide and an additional organic salt of iron, exposing portions of the coated surface to light, applying to said surface a solution of ferric ammonium oxalate, potassium ferricyanide and water, the volume of the ferric ammonium oxalate exceeding the combined volumes of the other two ingredients.

5. The method of making non-bleeding photoprints comprising coating a sheet of

material with potassium ferricyanide and ferric ammonium oxalate, exposing portions of the coated surface to light, applying to said surface a developing solution and thereafter washing, said developing solution comprising 70 1 pound potassium ferricyanide in 1 gallon of water and 5½ pounds ferric ammonium oxalate in 2 gallons of water.

6. The method of producing non-bleeding photoprints comprising sensitizing paper with a coating of a soluble ferricyanide and a soluble ferric compound, exposing a portion of the sensitized surface to actinic rays to reduce the trivalent iron ions of the exposed portion of the coating to divalent iron ions, treating the sensitized surface with an iron containing developer having present a ferricyanide and a ferric compound dissociating into trivalent iron ions, the latter reacting simultaneously with substantially all of the divalent iron ions to produce water insoluble iron compounds and thereby prevent bleeding on subsequent washing, and thereafter washing said paper to remove the soluble salts and obtain sharp definition between the exposed and unexposed portion of the sensitized surface.

7. The method of producing non-bleeding photoprints comprising sensitizing paper with a coating of a soluble ferricyanide and a soluble ferric organic compound, exposing a portion of the sensitized surface to actinic rays to reduce the trivalent iron ions of the exposed portion of the coating to divalent iron ions, treating the sensitized surface with an iron containing developer containing a ferricyanide and a ferric compound dissociating into trivalent iron ions adapted to simultaneously react with substantially all of the divalent iron ions and form water insoluble iron compounds acting to prevent bleeding on subsequent washing, and thereafter washing said paper to remove the soluble salts and obtain sharp definitions between the exposed and unexposed portions of the sensitized surface.

8. The method of producing non-bleeding photoprints comprising sensitizing paper with a coating of a soluble ferricyanide and a soluble ferric organic compound, exposing a portion of the sensitized surface to actinic rays to reduce the trivalent iron ions of the exposed portion of the coating to divalent iron ions, treating the sensitized surface with an iron containing developer having present a ferricyanide and an inorganic ferric compound dissociating into trivalent iron ions adapted to simultaneously react with substantially all of the divalent iron ions to form water insoluble iron compounds acting to prevent bleeding on subsequent washing, and thereafter washing said paper to remove the soluble salts and obtain sharp definition between the exposed and unexposed portions of the sensitized surface.

9. The method of producing non-bleeding photoprints comprising sensitizing paper with a coating of a soluble ferricyanide and a soluble ferric compound, exposing a portion of the sensitized surface to actinic rays to reduce the trivalent iron ions of the exposed portion of the coating to divalent iron ions, treating the sensitized surface with an iron containing developer having present a ferricyanide and a ferric compound dissociating into trivalent iron ions, the latter reacting simultaneously with substantially all of the divalent iron ions to form a mixture of Turnbull's blue and Prussian blue and thereby preventing bleeding on subsequent washing, and thereafter washing said paper to remove the water insoluble salts and obtain sharp definition between the exposed and unexposed portions of the sensitized surface.
- 10 In testimony whereof, I have subscribed my name.

HAROLD J. BRUNK.

25

30

35

40

45

50

55

60